

[54] **METHOD FOR INHIBITING CORROSION OF METAL USING POLYSULFONE COMPOUNDS**[75] Inventors: **Susumu Harada; Masami Haruta; Tadashi Kato, all of Koriyama, Japan**[73] Assignee: **Nitto Boseki Co., Ltd., Fukushima, Japan**[22] Filed: **Jan. 24, 1973**[21] Appl. No.: **326,290**[30] **Foreign Application Priority Data**

July 26, 1972 Japan ..... 47-74747

[52] U.S. Cl. .... **21/2.5 R; 21/2.5 A; 21/2.7 R; 21/2.7 A; 252/8.55 E; 252/148; 252/149; 252/151; 252/391; 260/79.3 R; 260/79.3 A**[51] Int. Cl.<sup>2</sup> ..... **C23F 11/00; C23F 11/04; C23F 11/10; C23F 11/16**[58] **Field of Search** ..... **21/2.5 R, 2.7 R; 260/79.3 A; 252/391, 8.55 E, 148, 149, 151**[56] **References Cited**

## UNITED STATES PATENTS

2,750,340 6/1956 Gerhardt et al. ..... 252/391

|           |         |                    |             |
|-----------|---------|--------------------|-------------|
| 2,938,034 | 5/1960  | Cislak .....       | 252/149     |
| 2,938,907 | 5/1960  | Rainey et al. .... | 252/391     |
| 3,121,091 | 2/1964  | Green .....        | 21/2.7 R    |
| 3,414,521 | 12/1968 | Teumac .....       | 21/2.7 R    |
| 3,502,578 | 3/1970  | Raifanider .....   | 21/2.5 R UX |
| 3,585,118 | 6/1971  | Harada et al. .... | 260/79.3 A  |
| 3,669,612 | 6/1972  | Annand et al. .... | 21/2.7 R    |
| 3,730,901 | 5/1973  | Knox et al. ....   | 21/2.7 R    |
| 3,809,655 | 5/1974  | Williams .....     | 252/391     |

*Primary Examiner*—Barry S. Richman*Assistant Examiner*—Bradley R. Garris*Attorney, Agent, or Firm*—Karl W. Flocks

## [57]

**ABSTRACT**

A metal corrosion inhibitor consisting of a polysulfone compound obtained by copolymerizing or interpolymerizing sulfur dioxide and at least one 1,6-diene compound. The above metal corrosion inhibitor may be added in a corrosion-inhibitorily effective amount, preferably at least 1 ppm., to a corrosive medium, with which a metal comes into contact, to inhibit the medium from corroding the metal.

**6 Claims, No Drawings**

**METHOD FOR INHIBITING CORROSION OF METAL USING POLYSULFONE COMPOUNDS**

This invention relates to a corrosion inhibitor for metals in water, aqueous solutions of salts or aqueous solutions of inorganic or organic acids, and to a method for inhibiting the corrosion of the metals with said inhibitor.

Corrosion of steel members in various coolers due to the oxygen or carbon dioxide dissolved in cooling water in recycle systems has resulted in severe troubles. Various methods have been proposed for the inhibition of such corrosion.

Various corrosion inhibitors have also been proposed for inhibiting the corrosion of metals caused by acid solutions used in the cleaning of metal surfaces, which is carried out for the removal of scales which stick to inner parts of an evaporator or boiler or for the pre-treatment of platings.

Furthermore, various inhibitors have been proposed for decreasing the loss of steel, reducing the amount of acid required and obtaining beautiful finished surface in pickling metals, especially, steel.

This invention provides a metal corrosion inhibitor represented by the general formula:



wherein M is at least one member selected from the group consisting of



in which  $\text{R}_1$  and  $\text{R}_2$ , which may be the same or different, are hydrogen, straight or branched chain alkyls having 1 to 18 carbon atoms, aryls having 6 to 24 carbon atoms, aralkyls having 7 to 25 carbon atoms, carboxymethyl, carboxyethyl, cyanomethyl, 2-cyanoethyl, 2-sulfoethyl, sulfopropyl, 2-hydroxyethyl, 3-chloro-2-hydroxypropyl, allyl, propargyl or  $\alpha$ - or  $\beta$ -naphthomethyl; and X is Cl, Br, I,  $\text{HCOO}$ ,  $\text{CH}_3\text{COO}$ ,  $\text{H}_2\text{PO}_4^-$ ,  $\text{HSO}_4^-$ ,  $\text{HSO}_3^-$ ,  $\text{CH}_3\text{SO}_4^-$ ,



or  $\text{HOCH}_2\text{COO}$ ,



5  
10  
15  
20

2  
in which Y is  $\text{CH}_2$  or O; and X is the same as defined regarding formula (I),



15

in which  $\text{R}_3$  is hydrogen, a straight or branched chain alkyl having 1 to 12 carbon atoms, hydroxymethyl, 2-hydroxyethyl, 3-hydroxypropyl, 4-hydroxybutyl,  $\text{NH}_2$ , chloromethyl or a group represented by formula (III-A):



25

30

in which  $\text{R}_4$ ,  $\text{R}_5$  and  $\text{R}_6$ , which may be the same or different, are hydrogen, straight or branched chain alkyls having 1 to 12 carbon atoms, aralkyls having 7 to 9 carbon atoms or 2-hydroxyethyl, including the case where



means



40  
45  
50  
55  
60  
65



and the case where



means



and X is the same as defined regarding the formula (I), or by formula (III-B):



in which R<sub>7</sub> and R<sub>8</sub>, which may be the same or different, are straight or branched chain alkyls having 1 to 6 carbon atoms, aralkyls having 7 to 9 carbon atoms or 2-hydroxyethyl; and X is the same as defined regarding the formula (I),



in which R<sub>9</sub> is hydrogen, a straight or branched chain alkyl having 1 to 18 carbon atoms, an aralkyl having 7 to 25 carbon atoms, 2-hydroxyethyl, allyl or propargyl; and X is the same as defined regarding the formula (I),



$\alpha$  is an average molar fraction of the SO<sub>2</sub> component in the general formula and ranges from 0.1 to 0.5; and n is a degree of polymerization. This invention also provides a method for inhibiting the corrosion of a metal which comprises adding a corrosion-inhibitorily effec-

tive amount of said metal corrosion inhibitor to a corrosive medium with which the metal contacts.

The metal corrosion inhibitor of this invention is a polysulfone obtained by copolymerizing or interpolymerizing sulfur dioxide and at least one compound selected from the group consisting of compounds represented by the following formulas (A) – (H):



The compounds represented by the general formulas (A) to (H) are all 1,6-diene type unsaturated compounds and generally, these are easily copolymerized with sulfur dioxide to produce polysulfones which are 1:1 cyclocopolymers. A number of these polysulfones have been disclosed by the inventors. (Refer to Japanese Pat. Publication No. 14587/66; U.S. Pat. No. 3,375,233 and 3,585,118; British Pat. Nos. 1,098,500 and 1,275,157; and Preprint IV at the 26th Annual Meeting of the Japan Chemical Society, P. 1820 (1972)).

For example, the copolymerization of the compounds represented by the formula (I) with sulfur dioxide results in polysulfones having the following structure:



In the present invention, it is necessary that in the polysulfone compound as the metal corrosion inhibitor, the sulfur dioxide component be contained in a molar fraction of at least 0.1. When the amount of the sulfur dioxide component is smaller, there is substantially no difference in corrosion-inhibiting effect between such a polysulfone compound and a polymer free from the sulfur dioxide component. In other words, in such a smaller amount of the sulfur dioxide component, there is seen substantially no enhancement of effect as corrosion inhibitor by copolymerizing sulfur dioxide. In the corrosion inhibitor of this invention, the maximum amount of the sulfur dioxide component is a molar fraction of 0.5, the preferable amount is a molar fraction of 0.3 to 0.5, and the most preferable amount is a molar fraction of 0.5. The term "molar fraction" used herein refers to an average value, and hence, each single molecule may contain the sulfur dioxide component in an amount outside the above-mentioned range.

In the preparation of the polysulfone compound as the corrosion inhibitor, sulfur dioxide is very easily copolymerized with at least one monomer having formulas (A) to (H) corresponding to the M component of the above general formula, and the sulfur dioxide and the above monomer or monomers are alternately bonded to each other to form an alternating copolymer as mentioned above. Where the above monomer or monomers (A) to (H) are used in excess of sulfur dioxide in the copolymerization, it is considered that an alternating copolymer or interpolymer in which the M component, i.e. the monomer or monomers, and the sulfur dioxide component are present in equimolar amounts is mainly formed, and a homopolymer or copolymer composed only of the M component based on the excessive monomer or monomers is partly formed, and simultaneously, a block copolymer consisting of the block of an alternating copolymer of the M component and the sulfur dioxide component and the block of a polymer composed only of the M component is also partly formed. Accordingly, where the monomers (A) to (H) corresponding to the M component are used in excess of sulfur dioxide, the corrosion inhibitor of this invention is a mixture of these polymers. However, in general, it is very difficult to isolate each copolymer from the mixture, and hence, examples in the case of an excess of the M component will hereinafter be illustrated in the form of a mere copolymer, and molar fractions of the respective components will be indicated.

Causes of corrosion of metals in an aqueous solution vary depending upon the kind of the solution, namely, the kind of substances dissolved therein, temperature and the kind of the metals. For example, the main causes of corrosion of metals in industrial water are considered to be the oxygen and carbon dioxide dissolved in water, and in the case of pickling solutions, corrosion is, of course, caused by acids. Effective corrosion inhibitors are determined depending upon the kinds of substances which cause corrosion, and even if the substances which cause corrosion are the same, effective inhibitors also vary when the temperature used is different. Furthermore, inhibitors to be added to pickling baths must meet various requirements, e.g., they should not lower the speed of removal of scales, they must result in a beautiful finished surface and they must have an excellent solubility and stability in the bath. In view of these requirements, the corrosion inhibitors must be "tailor made".

The polysulfone compounds used in this invention have the following general characteristics as corrosion inhibitors for metals:

1. Usually, low molecular weight compounds have been used as corrosion inhibitors, but the polysulfones used in this invention are high molecular weight compounds (corresponding to intrinsic viscosities of 0.01 to 2.0 dl/g as measured in N/10 NaCl solution at 30°C). (Conventionally, some of high molecular weight compounds have been used and it has been known that the high molecular weight compounds, even when used in an extremely smaller amount than low molecular weight compounds containing the same functional groups as those of said high molecular weight compounds, can exhibit the same corrosion inhibiting effect as the low molecular weight compounds.)
2. The polysulfone compounds used in this invention include a great number of compounds which have a common basic skeleton, but have different side chains. Moreover, any two or more compounds represented by the general formulas (I) to (V) may be copolymerized with sulfur dioxide into interpolymers, and hence, such inhibitors as having different two or more functional groups in one molecule are obtained. Therefore, suitable polysulfones may be chosen depending upon corrosion environment.
3. The polysulfone compounds are exceedingly stable in acids. Therefore, the corrosion inhibiting effect can be maintained for a long period of time when the compounds are used in acids, e.g., in the pickling of steel.

The polysulfone compound of this invention per se can act as a metal corrosion inhibitor, and therefore, it is generally added alone to a corrosive medium. However, it may be added along with an anticorrosive or synergistic agent which is known in the art, such as alkali halides, low molecular weight organic amine compounds and acetylene alcohol.

The amount of the polysulfone compounds added to a corrosion bath varies depending upon the kind of the compounds and corrosion environment, but generally, they may be used in an extremely low concentration. The addition in an amount of 1 ppm. to a corrosion bath can attain a considerable corrosion inhibiting effect, but usually they are used in a concentration higher than 5 ppm.

As mentioned before, the polysulfone compounds used in this invention include a great number of compounds, and the representatives thereof are as follows, and the corrosion inhibiting effects of thirty of these compounds will be specifically explained in the Examples given hereinafter:



(Dimethyldiallylammonium chloride- $\text{SO}_2$  copolymer)  
Intrinsic viscosity  $[\eta] = 0.12 \text{ dl/g}$  as measured in N/10 NaCl solution at 30°C. (The intrinsic viscosities of the

following compounds were measured in the same way as mentioned before unless otherwise specified.)



(Methyldiallylamine hydrochloride-SO<sub>2</sub> copolymer) [η] = 0.08 dl/g

(Methylbenzyldiallyl ammonium chloride-SO<sub>2</sub> copolymer) [η] = 0.14 dl/g



(Methylpropargyldiallyl chloride-SO<sub>2</sub> copolymer) [η] = 0.28 dl/g



(Diallylamine sulfate-SO<sub>2</sub> copolymer) [η] = 0.21 dl/g



(Diallylmorpholinium chloride-SO<sub>2</sub> copolymer) [η] = 0.12 dl/g



(Methylethyldiallyl ammonium paratoluenesulfonate-SO<sub>2</sub> copolymer) [η] = 0.14 dl/g



(Methyldiallylcarboxymethylammonium inner salt-SO<sub>2</sub> copolymer) [η] = 0.04 dl/g



(Diallylpiperidinium chloride-SO<sub>2</sub> copolymer) [η] = 0.14 dl/g



(Methyl-n-amylldiallyl ammonium chloride-SO<sub>2</sub> copolymer) [η] = 0.14 dl/g



(Cyclohexyldiallylamine acetate-SO<sub>2</sub> copolymer) [η] = 0.08 dl/g



[(3-Chloro-2-hydroxy)propylmethylldiallyl ammonium chloride-SO<sub>2</sub> copolymer] [η] = 0.15 dl/g



[N-(cyanoethyl)-diallylamine formate-SO<sub>2</sub> copolymer] [η] = 0.06 dl/g



(2-Hydroxyethylidiallylamine glycolate- $\text{SO}_2$  copolymer)  $[\eta] = 0.06 \text{ dl/g}$



[15]

5

10



[18]

(Diallylhydroxypropionic acid amide- $\text{SO}_2$  copolymer)  $[\eta] = 0.64 \text{ dl/g}$  as measured in DMSO at 30°C.



[16]

15

20

25

30

35

(Diallylaminocarbomethyldimethylsulfonium chloride- $\text{SO}_2$  copolymer)  $[\eta] = 0.32 \text{ dl/g}$



[19]

(Diallylaminocarbomethyltrimethylammonium chloride- $\text{SO}_2$  copolymer)  $[\eta] = 0.45 \text{ dl/g}$



[17]

30

35

(Hydroxyethylidiallylsulfonium chloride- $\text{SO}_2$  copolymer)  $[\eta] = 0.08 \text{ dl/g}$



[20]

$[\eta] = 0.14 \text{ dl/g}$

(Diallylaminocarbomethylpyridinium chloride- $\text{SO}_2$  copolymer)  $[\eta] = 0.26 \text{ dl/g}$

55

The suffixes outside the parentheses in the above formula indicate approximate molar fraction of each component. (The same is applied to the following formulas.)



[21]

$[\eta] = 0.21 \text{ dl/g}$



[22]

$[\eta] = 0.09$   
dl/g



[23]

$[\eta] = 0.4$  dl/g



[24]

$[\eta] = 0.14$   
dl/g

(N,N-diallyl urea)



[25]

$[\eta] = 0.21$   
dl/g

(N,N-diallyl cyanamide)



[26]

$[\eta] = 0.08$   
dl/g

(Diallylsulfoxide)



[27]

$[\eta] = 0.21$   
dl/g

(N,N-diallylthiourea)



[28]

$[\eta] = 0.16$   
dl/g

(N,N-diallylformamide)

13



14

[29]

$$[\eta] = 0.13 \text{ dl/g}$$



$$[\eta] = 0.08 \text{ dl/g}$$



[31]



[32]

These polysulfone compounds having the above structures (1) to (30) can be prepared by the method already disclosed by the inventors (see Japanese Pat. Publications No. 14587/66 and No. 31842/71; U.S. Pat. No. 3,375,233 and 3,585,118; British Pat. Nos. 1,098,500 and 1,275,157 and Preprint IV at the 26th Annual Meeting of the Japan Chemical Society, p. 1820 (1972)), or by similar methods. However, in general, the polysulfone compounds used in this invention may have a low degree of polymerization, and those having a degree of polymerization higher than 50 are not especially required. Therefore, the copolymerization is usually carried out in water.

The following examples illustrate some specific embodiments of this invention. It is to be understood, however, that this invention is in no way limited to the examples.

#### EXAMPLE 1

This example illustrates the effect of the corrosion inhibitors of this invention against corrosion of a mild steel piece in city water.

Stand-still tests were carried out for 100 hours at 20°C using a polished mild steel plate [JIS (abbreviation of Japanese Industrial Standards) G3141 - SPCCB 60 80 × 20 × 1 mm] as a test panel to examine the effects of corrosion inhibitors. The results are shown in Table 1, in which the corrosion inhibiting rate was calculated from the following formula:

$$65 \quad \frac{\left( \frac{\text{Degree of corrosion when no corrosion inhibitor is added}}{\text{Degree of corrosion when corrosion inhibitor is added}} \right)}{\left( \frac{\text{Degree of corrosion when no corrosion inhibitor is added}}{\text{Degree of corrosion when corrosion inhibitor is added}} \right)} \times 100 = \%$$

Table 1

| Corrosion inhibitors               | Poly-sulfone (1) | " (4) | " (8) | " (12) | " (17) | " (18) | " (21) | " (22) | " (24) | " (26) | " (29) | Dodecyl-trimethylammonium chloride (comparative example) |    |
|------------------------------------|------------------|-------|-------|--------|--------|--------|--------|--------|--------|--------|--------|----------------------------------------------------------|----|
| Concentration (ppm)                | 10               | 10    | 10    | 10     | 10     | 10     | 10     | 10     | 10     | 5      | 10     | 5                                                        | 10 |
| Corrosion inhibitor efficiency (%) | 82.4             | 88.4  | 96.5  | 82.5   | 96.5   | 95.3   | 92.6   | 89.5   | 95.4   | 89.5   | 92.4   | 34.2                                                     |    |

Test panel: Polished mild steel plate (JIS, G3141-SPCCB 80 × 20 × 1 mm).

Corrosive liquid: City water

Amount of liquid: 5 cc per cm<sup>2</sup> of the steel plate

Treatment: At 20°C for 100 hours.

## EXAMPLE 2

The same test panel as in Example 1 was subjected to corrosion treatment in city water under agitation at about 50°C for 100 hours. The results are shown in Table 2.

## EXAMPLE 3

The same test panel as in Example 1 was subjected to corrosion treatment in 10 % hydrochloric acid at 20°C for 100 hours. The results are shown in Table 3.

Table 2

| Corrosion inhibitors               | Poly-sulfone (2) | " (4) | " (6) | " (8) | " (11) | " (13) | " (15) | " (16) | " (19) | " (20) | " (22) | Dodecyl-trimethylammonium chloride (comparative example) |
|------------------------------------|------------------|-------|-------|-------|--------|--------|--------|--------|--------|--------|--------|----------------------------------------------------------|
| Concentration (ppm)                | 60               | 50    | 50    | 50    | 50     | 50     | 50     | 50     | 50     | 50     | 50     | 50                                                       |
| Corrosion inhibitor efficiency (%) | 91.4             | 91.5  | 92.4  | 94.1  | 90.8   | 88.6   | 89.4   | 93.5   | 94.6   | 91.5   | 92.0   | 62.5                                                     |

Test panel: Polished mild steel plate (JIS, G3141-SPCCB 80 × 20 × 1 mm).

Corrosive liquid: City water

Amount of liquid: 5 cc per cm<sup>2</sup> of the steel plate

Treatment: At 50°C ± 2°C for 100 hours with agitation

Table 3

| Corrosion inhibitors               | Comparative inhibitor (A)* | Comparative inhibitor (B)** | Poly-sulfone (1) | " (1)  | " (2)  | " (5)  | " (7)  | " (9)  | " (9)  | " (10) | " (11) | " (16) |
|------------------------------------|----------------------------|-----------------------------|------------------|--------|--------|--------|--------|--------|--------|--------|--------|--------|
| Concentration (ppm)                | 10                         | 10                          | 2                | 10     | 5      | 10     | 10     | 5      | 10     | 10     | 10     | 5      |
| Corrosion inhibitor efficiency (%) | 82.4                       | 2.5                         | 91.5             | 92.6   | 90.4   | 92.4   | 94.5   | 98.4   | 99.1   | 96.2   | 93.5   | 98.4   |
| Corrosion inhibitors               | Poly-sulfone (17)          | " (18)                      | " (20)           | " (20) | " (21) | " (22) | " (23) | " (25) | " (27) | " (28) | " (29) | "      |
| Concentration (ppm)                | 5                          | 10                          | 10               | 10     | 5      | 2      | 5      | 5      | 5      | 5      | 5      | 2      |
| Corrosion inhibitor efficiency (%) | 98.4                       | 90.6                        | 94.5             | 98.2   | 94.5   | 93.5   | 94.4   | 92.8   | 93.9   | 96.4   | 95.8   |        |

\*Comparative inhibitor (A) was a homopolymer of dimethyldiallyl ammonium chloride having the formula:



\*\*Comparative inhibitor (B) was dodecyltrimethylammonium chloride.

Test panel: Polished mild steel plate (JIS, G3141-SPCCB, 80 × 20 × 1 mm).

Corrosive liquid: 10 % hydrochloric acid.

Amount of liquid: 5 cc per cm<sup>2</sup> of the steel plate.

Treatment: At 20°C for 100 hours.

## EXAMPLE 4

The same test panel as in Example 3 was subjected to corrosion treatment in 10 % hydrochloric acid at 50°C for 2 hours to examine the corrosion inhibiting effect of polysulfones. The results are shown in Table 4.

## EXAMPLE 6

Mild steel plates with scale (JIS, G3101, 50 × 50 × 2.3 mm) as test panel were subjected to pickling treatment with hydrochloric acid and sulfuric acid under the following conditions:

Table 4

| Corrosion inhibitors               | Comparative sample (A)* | Comparative sample (B)** | Poly-sulfone (1) | " (2)  | " (5)  | " (7)  | " (9)  | " (9)  | " (10) | " (11) | " (16) | " (16) |
|------------------------------------|-------------------------|--------------------------|------------------|--------|--------|--------|--------|--------|--------|--------|--------|--------|
| Concentration (ppm)                | 10                      | 10                       | 10               | 5      | 10     | 10     | 5      | 10     | 10     | 10     | 5      | 10     |
| Corrosion inhibitor efficiency (%) | 78.6                    | 53.1                     | 86.5             | 84.8   | 87.8   | 89.6   | 94.6   | 98.9   | 96.6   | 94.8   | 96.5   | 98.1   |
| Corrosion inhibitors               | Poly-sulfone (17)       | " (18)                   | " (19)           | " (20) | " (21) | " (24) | " (26) | " (27) | " (28) | " (29) | " (30) |        |
| Concentration (ppm)                | 5                       | 10                       | 10               | 10     | 10     | 10     | 5      | 10     | 5      | 5      | 5      |        |
| Corrosion inhibitor efficiency (%) | 96.9                    | 98.6                     | 96.5             | 98.2   | 94.6   | 95.4   | 94.6   | 93.1   | 94.2   | 95.6   | 96.4   |        |

\* The same sample as in Table 3.

\*\*The same sample as in Table 3.

Test panel: The same test panel as in Table 3.

Corrosive liquid: 10 % hydrochloric acid.

Amount of liquid: 5 cc per cm<sup>2</sup> of the steel plate.

Treatment: At 50°C for 2 hours.

## EXAMPLE 5

The same test panel as in Example 1 was subjected to corrosion treatment in 10 % sulfuric acid at 20°C for 100 hours to examine the corrosion inhibiting effect of polysulfones. The results are shown in Table 5.

25 % sulfuric acid + 5 % ferrous ion (added as ferrous sulfate) at 98 ± 1°C for 3 minutes.

8 % hydrochloric acid + 7 % ferrous ion (added as ferrous chloride) at 85 ± 1°C for 3 minutes.

Amount of liquid: 350 g of the acid per 2 test panels.

The results are shown in Table 6, wherein the descal-

Table 5

| Corrosion inhibitors               | Poly-sulfone (1)  | " (3)  | " (4)  | " (4)  | " (4)  | " (6)  | " (9)  | " (12) | " (13) | " (14) | " (16) | "                                                        |
|------------------------------------|-------------------|--------|--------|--------|--------|--------|--------|--------|--------|--------|--------|----------------------------------------------------------|
| Concentration (ppm)                | 100               | 100    | 10     | 50     | 100    | 50     | 20     | 20     | 50     | 50     | 50     | 50                                                       |
| Corrosion inhibitor efficiency (%) | 84.5              | 91.4   | 86.5   | 92.5   | 96.5   | 92.4   | 94.6   | 93.7   | 89.6   | 86.5   | 87.2   |                                                          |
| Corrosion inhibitors               | Poly-Sulfone (16) | " (17) | " (17) | " (20) | " (20) | " (21) | " (23) | " (25) | " (26) | " (27) | " (28) | Dodecyl-trimethylammonium chloride (comparative example) |
| Concentration (ppm)                | 100               | 20     | 50     | 20     | 50     | 20     | 20     | 50     | 50     | 50     | 50     | 100                                                      |
| Corrosion inhibitor efficiency (%) | 96.5              | 89.5   | 94.2   | 86.5   | 96.4   | 94.5   | 96.2   | 94.5   | 93.6   | 96.8   | 96.8   | 49.6                                                     |

Test panel: Same as in Table 3.

Corrosive liquid: 10 % sulfuric acid.

Amount of liquid: 5 cc per cm<sup>2</sup> of the steel plate.

Treatment: At 20°C for 100 hours.

ing speed is expressed by the time required for the complete removal of mill scale on the surface of metal.

wherein  $R_1$  and  $R_2$ , which may be the same or different, are hydrogen, straight or branched chain alkyls having

Table 6

| Corrosion inhibitors                                    | Pickling liquid and pickling condition | Concentration of inhibitor (ppm) | Corrosion inhibitor efficiency (%) | Descaling speed (second) | Pickling liquid and pickling conditions | Concentration of inhibitor (ppm) | Corrosion inhibitor efficiency (%) | Descaling speed (second) |
|---------------------------------------------------------|----------------------------------------|----------------------------------|------------------------------------|--------------------------|-----------------------------------------|----------------------------------|------------------------------------|--------------------------|
| None                                                    |                                        | —                                | —                                  | 32                       |                                         | —                                | —                                  | 29                       |
| Polysulfone 1                                           |                                        | —                                | —                                  | —                        |                                         | 20                               | 84.5                               | 32                       |
| 2                                                       |                                        | —                                | —                                  | —                        |                                         | 20                               | 82.5                               | 32                       |
| 3                                                       |                                        | 90                               | 86.5                               | 34                       |                                         | —                                | —                                  | —                        |
| 4                                                       |                                        | 90                               | 84.2                               | 34                       |                                         | —                                | —                                  | —                        |
| 5                                                       |                                        | 90                               | 89.5                               | 38                       |                                         | 20                               | 84.2                               | 32                       |
| 7                                                       | 25 % $H_2SO_4$                         | 90                               | 90.4                               | 39                       | 8 % HCl                                 | 20                               | 84.4                               | 33                       |
| 8                                                       | + 5 % $Fe^{++}$                        | 40                               | 78.6                               | 33                       | + 7 % $Fe^{++}$                         | 5                                | 81.0                               | 30                       |
| 9                                                       | 98 ± 1°C                               | 90                               | 90.5                               | 39                       | 85 ± 1°C                                | 20                               | 85.2                               | 33                       |
| 10                                                      | 3 minutes                              | 90                               | 83.6                               | 35                       | 5 minutes                               | 30                               | —                                  | —                        |
| 11                                                      |                                        | 90                               | 85.2                               | 35                       |                                         | 30                               | 86.3                               | 34                       |
| 12                                                      |                                        | 40                               | 76.5                               | 32                       |                                         | 10                               | 80.6                               | 32                       |
| 13                                                      |                                        | 90                               | 77.4                               | 32                       |                                         | 20                               | 82.2                               | 31                       |
| 14                                                      |                                        | 90                               | 88.5                               | 38                       |                                         | 20                               | 84.6                               | 31                       |
| 16                                                      |                                        | 40                               | 90.0                               | 40                       |                                         | 10                               | 81.5                               | 32                       |
| 17                                                      |                                        | 60                               | 91.6                               | 40                       |                                         | 20                               | 82.5                               | 31                       |
| 18                                                      |                                        | 90                               | 92.0                               | 41                       |                                         | 20                               | 83.6                               | 32                       |
| 19                                                      | 25 % $H_2SO_4$                         | 90                               | 91.2                               | 40                       | 8 % HCl                                 | 30                               | 84.1                               | 33                       |
| 20                                                      | + 5 % $Fe^{++}$                        | 90                               | 90.8                               | 39                       | + 7 % $Fe^{++}$                         | 20                               | 86.2                               | 33                       |
| 25                                                      | 98 ± 1°C                               | 90                               | 79.6                               | 36                       | 85 ± 1°C                                | 30                               | 80.1                               | 31                       |
| 26                                                      | 3 minutes                              | 90                               | 89.6                               | 37                       | 5 minutes                               | 20                               | 84.2                               | 32                       |
| 27                                                      |                                        | 90                               | 92.1                               | 40                       |                                         | 20                               | 87.6                               | 34                       |
| 28                                                      |                                        | 90                               | 86.8                               | 35                       |                                         | 20                               | 83.6                               | 32                       |
| 29                                                      |                                        | 50                               | 82.8                               | 36                       |                                         | 10                               | 79.4                               | 31                       |
| 30                                                      |                                        | 80                               | 83.5                               | 34                       |                                         | 20                               | 86.4                               | 34                       |
| Dodecytri-methylammonium chloride (comparative example) |                                        | 100                              | 45.3                               | 42                       |                                         | 30                               | 40.5                               | 36                       |

## EXAMPLE 7

Copper wires which had discolored to brown in the air were dipped in a 1 % aqueous solution of hydrochloric acid containing 100 ppm of polysulfone (8) or (27) at 60°C for 30 seconds, and then rinsed with water. Thereafter, the thus treated wires were allowed to stand at 30°C and at a relative humidity of 100 %. The copper wire treated with hydrochloric acid containing polysulfone (8) showed no change for 3 days and the copper wire treated with hydrochloric acid containing polysulfone (27) showed no change for 5 days. On the other hand, a copper wire which was treated with 1 % hydrochloric acid aqueous solution containing no polysulfone in the same manner as mentioned above was discolored to brown after the lapse of 2 hours.

What is claimed is:

1. A method for inhibiting the corrosion of a metal which comprises adding to a corrosive medium with which the metal comes into contact a corrosion-inhibitorily effective amount of a metal corrosion inhibitor represented by the general formula



wherein M is one member selected from the group consisting of



1 to 18 carbon atoms, aryls having 6 to 24 carbon atoms, aralkyls having 7 to 25 carbon atoms, carboxymethyl, carboxyethyl, cyanomethyl, 2-cyanoethyl, 2-sulfoethyl, sulfopropyl, 2-hydroxyethyl, 3-chloro-2-hydroxypropyl, allyl, propargyl or  $\alpha$ - or  $\beta$ -naphthomethyl; and X is Cl, Br, I,  $HCOO$ ,  $CH_3COO$ ,  $H_2PO_4$ ,  $HSO_4$ ,  $HSO_3$ ,  $CH_3SO_4$ .



or  $HOCH_2COO$ , and



55

60

65

66

wherein X is the same as defined above and Y is  $CH_2$  or O;  $\alpha$  is an average molar fraction of the  $SO_2$  component in the general formula and ranges from 0.1 to 0.5; and n is a degree of polymerization.

2. A method according to claim 1, wherein the corrosive medium is water, an aqueous salt solution or an inorganic or organic acid.

**21**

3. A method according to claim 1, wherein the metal corrosion inhibitor is added in an amount of at least 1 ppm to the corrosive medium.
4. A method according to claim 3, wherein the corrosive medium is water, an aqueous salt solution or an inorganic or organic acid.
5. A method according to claim 1, wherein the metal

corrosion inhibitor is added in an amount of at least 5 ppm to the corrosive medium.

6. A method according to claim 5, wherein the corrosive medium is water, an aqueous salt solution or an inorganic or organic acid.

\* \* \* \* \*

10

15

20

25

30

35

40

45

50

55

60

65